

**UNITED STATES PATENT OFFICE**

2,680,057

# CYCLOPROPYL QUATERNARY AMMONIUM COMPOUNDS AND PROCESS OF APPLYING TO TEXTILES

John R. Janes, Garden City, N. Y., assignor to  
Deering Milliken Research Trust, Greenwich,  
Conn., a nonprofit trust of Maine

No Drawing. Application August 31, 1948,  
Serial No. 47,150

7 Claims. (Cl. 8—116.2)

1

This invention relates to textile finishing compounds, to a process of treating textile materials in order to improve their properties and to the improved textile materials thereby produced.

Cellulosic, proteinaceous and other textiles have heretofore been rendered water repellent by treating them with water repellent quaternary ammonium compounds containing a long chain aliphatic radical. These compounds are believed to react chemically with the textile, but have only one reactive functional group. It has now been ascertained that if like compounds are prepared containing two unlike functional groups, each of which are capable of reacting with the textile molecule, additional modifications of the physical properties may be obtained. Such modifications include dimensional stability and crease-resistance.

Thus in accordance with this invention, textile materials are treated with quaternary ammonium salts of cyclopropane derivatives. These compounds have a radical containing a cyclopropyl group linked to the quaternary nitrogen atom and are capable of reacting with the textile molecule at both the cyclopropane and the quaternary ammonium groups. The compounds increase the water repellency of textile materials while at the same time softening them and enhancing their dyeing properties, and usually impart dimensional stabilization or shrinkage control and increase resistance to the material as well, possibly because of the formation of cross linkages between adjacent textile molecules or because of polymerization of the compound or its decomposition products *in situ* to form a resin.

## THE COMPOUNDS OF THE INVENTION

They have the following general formula:



where A is a bivalent or trivalent organic aliphatic, cycloaliphatic or aromatic radical, usually of not over 30 carbon atoms, and is selected from the group consisting of hydrocarbon radicals and radicals containing a linkage selected from the group consisting of ether, imino, carbonyl, carboxylic amide, carboxylic ester, substituted urea and substituted carbamate linkages, i. e., radicals containing one or several  $\text{—O—}$ , NH, CO, CONH, NHCO, CONR, COO, OCC, NHCONH, CONHCONH,  $\text{OCH}_2\text{NHCONH}$ ,  $\text{NHCOCH}_2\text{O}$ , NHCOO or OCONH linkages; and R is an alkyl radical. Typical hydrocarbon rad-

2

icals are methylene, ethylene, octamethylene, octadecylene, decamethylene, benzene, naphthalene, cyclohexane and cyclopentane.

X is an inorganic or organic anion, such as chloride, bromide, iodide, acetate, formate, thiocyanate, nitrate, sulfate, or nitrite.

$N(tert)$  is the residue of a tertiary amine. Typical tertiary amine residues include those in which three nitrogen valences are taken up in one ring, as in pyridine, pyrazine, pyrimidine, quinoline, isoquinoline, acridine, and phenanthridene, those in which two nitrogen valences are taken up in one ring, as in piperidine, or tetrahydroquinoline or isoquinoline, and a third taken up with an alkyl group, and those in which three valences are taken up with alkyl groups such as methyl, ethyl, propyl, butyl, pentyl, and hexyl, whether  $n$ -, secondary or tertiary.

Within the generic formula set forth above,  
20 the compounds of the invention may, as can be  
seen from the subsequently presented examples,  
take the form:



Where R is a bivalent radical selected from the group consisting of

30  $\text{--O--}, \text{--CO--}, \text{--COO--}, \text{--CONH--}, \text{--CO--}, \text{--NHCOO--}$ ,  
 $\text{--NHCONH--}, \text{--CONHCONH--}, \text{--OCH}_2\text{NHCONH--}$   
 and

35 A is a hydrocarbon radical containing from 1 to 20 carbon atoms;  $m$ ,  $n$ , and  $p$  are numbers selected from the numbers 0 and 1, subject to the proviso that they cannot all be 0 at the same time  
40 and, further, that when  $m$  and  $n$  are both 1,  $p$  is also 1; N(tert) is a tertiary amine; and X is an anion.

When A is trivalent, the formula may assume one of these special forms:



where Z is a bivalent aliphatic, aromatic or cyclo-aliphatic radical, such as methylene, ethylene, butylene, hexylene, decamethylene, octadeca-

methylene, or a benzene, naphthalene, or cyclohexane residue.

These compounds may be prepared in a number of ways.

1.  $\alpha, \gamma$ -Halogen alkanes may be treated with metallic sodium in ether or with zinc in alcohol:



where Y=any organic radical such as one containing halogen, an N(tert)X group, or a group capable of chloromethylation, such as a terminal OH or CONH<sub>2</sub> group.

2.  $\alpha, \beta$ -Halogen alkanes may be treated with the sodium derivative of malonic ester:



The cyclopropionic acid may be used in various conventional syntheses to produce quaternary ammonium salts as shown in the examples. To illustrate, the corresponding amide may be formed, and the latter chloromethylated and treated with a tertiary amine.



Similarly, substituted ureas, carbamates and esters may be prepared.

3.  $\gamma$ -Halogenated nitriles may be treated with sodium amide in liquid ammonia, and then hydrolyzed to the acid or amide:



Treatment of the nitrile with sodium gives a dimer which may be hydrolyzed to a ketone:



This may be converted to the alcohol and chloromethylated as set forth above.

4. Allyl bromide may be treated with substituted alcohols and chlorine:



taining halogen, an N(tert)X group, or a group capable of chloromethylation.

These compounds are white or pale-colored viscous oils or solids, soluble or dispersible in water (benzene, chloroform, ethyl alcohol, carbon tetrachloride, and ethylene dichloride, sparingly soluble in ether and acetone. Most of the compounds are thoroughly stable even in aqueous solution, but some may decompose or polymerize gradually at room temperature after being dissolved in water.

The quaternary ammonium group of the compounds decomposes when heated above 100° C., the reaction being accomplished by liberation of the tertiary amine employed in its formation. The free radical liberated in this reaction, which is of the form:



may react with another free radical to form a dimer, or react with water to form a fatty alcohol. If the reaction was brought about in the presence of cellulose, it may react with a hydroxyl group of a cellulose molecule to form an ether of the general structure



Also, the free radical may decompose further since the cyclopropane ring may open and react either with the cellulose molecule to form an ether of the general structure



or with other cyclopropane residues to form a resin in or about the fibers. This makes possible the formation of cross links between adjacent cellulose molecules of the structure



When the compound contains only one cyclopropane and one quaternary ammonium group, linear polymers may be formed by interaction of the decomposition products; if the compound contains three or four functional groups, such as two cyclopropane and/or two quaternary ammonium groups, cross-linked polymers or linear polymers themselves linked to cellulose may be formed.

The particular A linkage may also influence the reaction. If A is an amide, carbamate, or urea residue, for example, polymerisation of the decomposition products is favored.

These postulated reactions are believed responsible for the permanent water repellency, dimensional stability and crease-resistance imparted by these compounds to cellulosic, proteinaceous and other textile materials.

This reaction takes place with cellulosic materials as a class regardless of their physical form whether fibers, roving, yarns, fabrics or films typical natural cellulosic materials including cotton, flax, jute, hemp, ramie, linen, sisal, bast and wood pulp. Reaction also occurs with artificial cellulosic films and fibers such as regenerated cellulose, cellulose acetate, cellulose acetate butyrate, cellulose propionate, cellulose acetate propionate and ethyl cellulose. Apparently chemical reactions occur with the protein molecule, probably at the NH group; the compounds react with

wool, silk, casein, albumen, alginate and like proteinaceous films or fibers, regardless of their stage of manufacture. They also give similar results with fibers formed from nylon, copolymers of vinyl chloride and vinyl acetate, such as are sold under the name "Vinyon," and copolymers of vinyl chloride and vinylidene chloride, such as are sold under the name "Saran."

When the compounds of the invention are applied to textile materials and then decomposed, it will be understood that any or all of the above chemical reactions may occur consecutively or simultaneously. Thus, the compound may react with the textile, polymerize in situ in the fiber or film to form a resin, and also react to form a dimer.

When the compounds of the invention are applied to textiles, the properties of the textile are modified depending upon the particular compound employed and the quantity of the compound deposited in or on the material. When the material contains between about 0.05 percent and about 20 percent by weight of the compound, its softness and water repellency are increased. The softest and most highly water repellent finishes are produced at between about 0.5 percent and about 10 percent compound by weight of the material. Best water repellent effects are obtained with compounds having a cyclorpropyl-containing radical equivalent in length to a 10 to 20 carbon straight-chain alkylene group. When the textile material contains between about 2 percent and about 20 percent by weight of certain compounds of the invention, particularly compounds having one or two cyclorpropyl-containing organic radicals equivalent in length to an 8 to 16 carbon straight chain alkylene group, its dimensions may be stabilized against either shrinking or stretching. Best stabilization is obtained at between about 5 percent and about 15 percent compound by weight of the material. Other textile finishing agents may be applied to the textile in order to further modify its properties as is described below.

#### THE PROCESS OF THE INVENTION

In brief, the textile material is treated with a solution or dispersion of a compound or mixture of compounds of the invention, the solvent wholly or partially removed by heat and/or in a vacuum and the material heated or baked for a time and at a temperature sufficient to cure it, that is, to bring about chemical reaction between the compound and the textile. If desired, curing may be carried out simultaneously with solvent removal or drying. The cured material may be washed to remove unreacted material and undesirable by-products of the reaction.

The conditions for carrying out the impregnation depend upon the nature of the material being treated, the compound and the concentration of the treating solution, and the type of finish desired. The compounds are ordinarily employed in the form of an aqueous solution or dispersion. However, if tightly woven fabrics are to be treated, it is frequently advantageous to add to the treating solution a small quantity of alcohol, acetone or a wetting agent of the cationic or nonionic type. Solutions of the compounds in organic liquids, such as benzene, ethyl alcohol, and ethylene dichloride, may also be employed.

The concentration of the treating solution depends upon the material being treated and the result desired. Soft finishes which impart only a small degree of water repellency are obtained

when the treating solution contains between about 0.1 percent and about 0.5 percent of the compound while highly water repellent soft finishes are obtained when the concentration is between about 0.5 percent and about 20 percent compound depending upon the structure of the compound employed. The material may also be rendered dimensionally stable by use of treating solutions of these concentrations. These figures are based on a 100 percent pickup of treating solution by weight of the fabric being treated. If a lower pickup is obtained, the concentration of the treating solution should be increased proportionately. This is particularly true, for example, when tightly woven fabrics are being treated.

In order to prevent or minimize loss in tensile strength and tendering when cellulosic materials are treated with the compounds of the invention, the pH of the treating solution should be adjusted so that the cured treated material has a pH between 5 and 8.0, preferably 6 and 7. The pH of the cured material is considered as equivalent to that of the water extract obtained by immersing 20 grams of the cured material in 500 cc. of water for one-half hour. In most cases it will be found that the cured material has a pH the same as or slightly more acid than the treating solution since the acid by-products of the chemical reaction between the material and the compound are usually volatile and are largely lost during curing. The pH of the treating solution therefore should be in the range of 5 to 10. Buffers, which preferably are non-volatile at the curing temperature used, and inert both to the compounds of the invention and to the textile material, are employed to maintain the pH of the treating solution at the desired value. Depending upon the pH of the initial treating solution, bases such as triethanolamine, diethanolamine, sodium acetate, ammonium acetate, pyridine, hexamethylene tetramine, and sodium formate, or acids such as lactic, glycolic or alpha-hydroxybutanoic acids may be used to adjust the pH of the initial solution.

Other textile finishing agents may be added to the treating solution to give a fuller or stiffer handle to the material. Substances such as ammonium acetate, carragheen moss, gum tragacanth, natural resins and waxes, ammonium stearate or water-soluble cellulose derivatives, such as methyl, hydroxyethyl and sodium carboxymethyl cellulose, may be added. Additional water repellent compounds may be added if desired. Preferably cationic quaternary ammonium compounds which are closely related to the compounds of the invention are employed, for example, octadecyloxymethylpyridinium chloride, N,N-di(chloropyridiniummethyl) paraphenylene di-carbamate, stearamidomethylpyridinium chloride and hexamethylene or decamethylene di(oxy-methylpyridinium chloride). Where these additional agents are insoluble in water, they are frequently dispersed in the treating solution by the quaternary ammonium compounds of the invention, which also have detergent properties.

The treating operation is preferably carried out at temperatures below 40° C. where the compounds of the invention are readily decomposed in aqueous or organic solvent solutions or dispersions. More stable compounds may be applied at more elevated temperatures, in some cases even at the boiling point, but even the most stable compounds tend to become acid when kept at such temperatures for any extended period of time;

and give a less satisfactory finish, not as resistant to organic solvents. In general, therefore, the treating operation is carried out at between 20° and 40° C.

The treatment is carried out by padding or soaking the material in the treating solution or dispersion. Conventional 2 or 3 roll padders may be used. The material is preferably subjected to pressure during or after treatment in order to insure thorough impregnation. Surplus liquor is removed by squeezing or hydroextracting. When the textile material is being dimensionally stabilized and/or crease-proofed, an effect obtained with certain of the compounds of the invention, particularly the urea derivatives, it is then stretched while still wet to the desired finished dimensions and then drying and baking are carried out while the material is under tension. This stretching step is unnecessary when the material is merely to be rendered water-repellent.

In this connection, it should be noted that the effects of the treatment are not always entirely fast to severe laundering. For this reason it is important that the treatment be applied to the fabric in its normal, relaxed state. After treatment and curing are carried out with an over-stretched fabric, then the latter will be stabilized at its extended size. When the stabilization effect is worn off on laundering the fabric will then shrink to its normal relaxed size. On the other hand, if the process is carried out on a fabric in its relaxed state, the gradual loss of finish during laundering will not cause shrinkage.

Many of the compounds of the invention are readily hydrolyzed by water at temperatures above about 80° C. Therefore, if the impregnated textile material is heated at temperatures above 80° C. while still wet, premature decomposition of the quaternary ammonium compound may occur, and no water repellency may thereafter be obtained. This is particularly true of thick or tightly woven fabrics which tend to retain moisture for a long period of time, even at elevated temperatures, thus facilitating the hydrolysis of the quaternary ammonium compound. In such cases, it is best to first dry the fabric thoroughly so that baking and curing may be carried out in the absence of moisture. The drying temperature is preferably between 30° and 80° C., but the temperature of drying is less important than the speed and other conditions. If the fabric is dried in more or less stagnant air as in an oven, without artificial circulation, it should not be submitted to a drying temperature of more than 30° C. When, on the other hand, it is dried in a blast of hot air so that the water may be removed rapidly, say in about 3 minutes, then the drying temperature may rise to 80° C. Again, when the treated material is dried on a steam-heated cylinder at 120° C., no permanent water repellency may be obtained.

The baking or curing treatment is essential to the development of permanent softness, water repellency, dimensional stabilization, and crease-resistance. The term "permanent" refers to the resistance of the finish to laundering and dry cleaning operations. A good finish may be obtained if the baking step is omitted, but it will not be permanent.

The curing or baking temperature should be between 80° and 200° C., preferably between 100° and 150° C. The time of baking is inversely proportional to the temperature used, and both depend to some extent on the nature of the com-

ound and of the textile material. A longer baking time and a relatively low temperature should be used with thick or tightly woven fabrics in order that the heating may be uniform throughout, while open weave fabrics may safely be heated for a very short time at a higher temperature. If tendering of the material is to be avoided, the time of baking is preferably kept as short as possible and the baking temperature as low as possible.

In the case of open weave fabrics, if a brisk circulation of air is provided around and through the material, the preliminary drying step may be omitted and the treated material heated at once at the baking or curing temperature.

The drying operation may be carried out in a covered tenter frame, while curing or baking is best carried out on a loom, mat, roll or air lay dryer.

20 After baking or curing, the material is given a light soap wash, preferably with the addition of a small proportion of base, such as ammonia, to remove undecomposed quaternary ammonium salt, together with any of its water-soluble decomposition or reaction products and buffer compounds. Frequently, no water-repellency or dimensional stability is apparent until this is done.

The new quaternary ammonium compounds may also be used in conjunction with synthetic 30 resins to make the textile material being treated crease-resistant. In conjunction with such materials, the compounds impart softness and suppleness, thus preventing the harshness and stiffness which results when the crease-resistant

35 agent is applied alone. A synthetic resin is formed in situ by impregnation of the textile material with a solution, usually aqueous, of a partially condensed resinous condensation product derived from an aldehyde or aldehyde-yielding substance, and urea, thiourea, or a derivative thereof, phenol, melamine or a derivative thereof, or with the components required to form such a resinous condensation product, with a subsequent heat treatment to insolubilize the resin.

40 Where aldehyde condensation products of urea or phenol are used, an acid or acid-yielding substance is employed as a catalyst. This may be omitted in the case of melamine aldehyde resins. The quaternary ammonium compound may be 45 added to the resin solution, or the textile treated therewith, before or after treatment with the resin.

#### Example 1

50 Pyridinium hydrochloride is prepared by dissolving pyridine in benzene, passing in dry, gaseous hydrogen chloride and filtering off and drying the precipitated salt.

A mixture containing one mole of the cyclopropyl carbinol ether of dimethylol urea, 100 55 parts of 95 percent ethyl alcohol and 1.2 moles of pyridinium hydrochloride is reacted at 70° C. for 30 minutes, giving a clear solution. The solution is evaporated at 40-50° C. to leave as a residue a water soluble product which is identified as 60 the pyridinium salt of cyclopropyl methyl ether of dimethylol urea,



70 Upon heating a sample of the dried powder at 100° C. fumes of pyridine are given off and an amorphous, water insoluble solid is obtained. An aqueous solution is even more rapidly and easily

dissociated when heated above 90° C. and deposits a water insoluble film on the bottom of a shallow dish containing the solution. Upon baking the dish at 135° C., this film is further converted to an infusible resin.

Ten parts by weight of the dried powder are dissolved in 30 parts of hot 95 percent ethyl alcohol and diluted with 100 parts of warm water. 80 x 80 cotton cloth and spun rayon challis cloth are padded in the solution, passed between rollers set to retain a weight of solution equal to the weight of the cloth, dried and cured by heating in an oven for 7 minutes at 135° C., washed 15 minutes in a one percent soap solution, dried and ironed. Both samples of treated cloth are then very soft and have excellent permanent water repellency, together with some crease resistance and shrinkage resistance.

#### Example 2

Dry hydrogen chloride gas is introduced into a mixture heated to 40° C. and containing one mole of cyclopropionamide, 150 g. of benzene and one mole of paraformaldehyde, until formation of the chloromethyl compound, which can be clearly recognized by the benzole solution becoming clear. The water from the reaction which accumulates at the bottom of the vessel is run off. The benzene and surplus hydrochloric acid are driven off in a vacuum and the chloromethyl compound obtained is stirred with 1.5 moles of pyridine. The precipitate which forms is separated and dried in vacuo.

The cyclopropionamido methylene pyridinium chloride is dissolved in water to give a 6 percent solution, whose pH is adjusted to 8.0 by addition of sodium phosphate solution. A 50-50 rayon-cotton cloth is padded with this solution to give a 100 percent pick-up by weight, dried at 70° C. for 15 minutes and then baked at about 130° C. for 5 minutes. The resulting product shows good and permanent water repellency.

#### Example 3

One mole of  $\omega$ -cyclopropyl decamethylene cyano is dissolved in 100 g. of benzene and one mole of paraformaldehyde added. The nitrile may be prepared from the corresponding acid by forming the amide and then reacting the latter with  $P_2O_5$ . Dry hydrogen chloride gas is introduced at ordinary room temperature until the chloromethyl imino ether is formed. The benzene and surplus hydrochloric acid are removed by suction in a vacuum at a temperature of about 40-50° C. and the chloromethyl compound then stirred with two moles of pyridine. The water soluble quaternary pyridinium salt of the chloromethyl imino ether is produced, of the formula



Wool sliver and viscose floc are treated in an aqueous 10 percent solution of this quaternary pyridinium salt. Following impregnation the material is dried at 50° C. and then subjected to a heat treatment at not over 135° C. The resulting products are permanently water repellent and dimensionally stable.

#### Example 4

To 250 parts of pyridine, 23 parts of dry hydrogen chloride gas are added. One mole of cyclopropylcarbamyl hexamethylene isocyanate (prepared by reacting cyclopropyl carbinol and hexa-

methylene diisocyanate) and one mole of paraformaldehyde are added and the mixture is stirred and heated at 70° C. until a test sample of the reaction mixture gives a clear solution in water.

The reaction mixture is cooled and ether is added, whereby the new compound is precipitated in colorless crystals. The compound has the formula,



A sufficient quantity of the compound is dissolved in water to give a 10 percent solution. A rayon fabric is padded with this solution at room temperature to a 100 percent pick-up by weight, dried at 75° C. for 30 minutes and then baked at 120° C. for 30 minutes. The resulting fabric shows a high degree of permanent water repellency, and some dimensional stability.

#### Example 5

To 130 parts of dry pyridine 40 parts of dry gaseous hydrogen chloride are added. One mole of paraformaldehyde and one mole of cyclopropionyl urea (prepared from urea and cyclopropionic acid) are then added and the mixture is stirred and heated at 70-75° C. until after about 18 hours a test sample gives a clear solution in warm water. The mixture is then cooled and acetone is added, whereby the new compound is precipitated as colorless crystals. It is readily soluble in water at 60-70° C. to give a clear, foaming solution. When this solution is kept hot, decomposition takes place, a precipitate is formed and the tendency to produce foaming is lost. The compound has the formula:



This compound is dissolved in water to give a 3 percent solution and a cotton cloth padded therewith to a 100 percent pick-up by weight. The cloth is then dried at 60° C. for one-half hour and baked at 90° C. for 5 minutes and then at not over 145° C. for 20 minutes. The resulting product shows a high degree of permanent water repellency, dimensional stability and crease-resistance.

#### Example 6

3.6 moles of hydroxy butyl urea (prepared from 1,4-butanediol and urea) is placed in a three-neck flask fitted with an addition funnel, stirrer and hydrochloric acid gas exit tube and cooled to 0° C. 2.3 moles of allyl bromide and chlorine are added simultaneously at such a rate that the mixture remains just on the green side while the temperature is held at about 0° C. Upon completion of the reaction, air is introduced to expel the hydrochloric acid; thereafter the balance of the acid is removed under vacuum with application of heat. The reaction mixture is then distilled under vacuum to recover the 1-chloro, 3-bromo, 2-butoxyurea propane.

To effect cyclization, about 19.5 grams of zinc dust are added with vigorous stirring to about 70 grams of water placed in a three-neck flask fitted with a funnel, stirrer and condenser, and the flask is heated to reflux temperature. 0.7 mole of the ether is added drop by drop and refluxing continued at a moderate rate. The product is extracted from the water layer with ethyl ether

and dried over sodium sulfate. The ether is then removed and the product recovered.

To 130 parts of dry pyridine dry hydrogen chloride is added. One half mole of paraformaldehyde and 0.5 mole of N-cyclopropyloxytetra methylene urea



are then added and the mixture is stirred and heated at 60-65° C. until a test portion gives a clear, foaming solution in warm water. The reaction mixture is then cooled and ether is added, whereby the new compound is precipitated in colorless, very hygroscopic crystals. This has the formula:



Sufficient compound is dissolved in water to produce a 4 percent solution, which is then padded on a 100 percent rayon fabric and on a 50 percent rayon-50 percent wool fabric to a 100 percent pickup by weight. Both cloths are then dried at 70-80° C. and baked at from 120 to 140° C. for 15 minutes. The resulting products are permanently water repellent and show good dimensional stability.

#### Example 7

200 parts of ethylene chlorohydrin and 220 parts of dry pyridine are heated together for 24 hours at 100° C., care being taken to exclude moisture. Into the hydroxyethyl pyridinium chloride thus produced one mole of



(cyclopropylauryl chloride) is allowed to run gradually while stirring, the reaction mixture being maintained continuously at water bath temperature. The reaction is continued until a sample is soluble in water to a clear solution. The product thus obtained is believed to have the formula:



The product is dissolved in water in sufficient quantity to give a 6 percent solution and the pH adjusted to 8.0 with triethanolamine. A viscose rayon fabric is padded with this solution to a 100 percent pick-up by weight, dried at 60° C. and baked at not over 140° C. for 10 minutes. The product shows a water repellency and shrinkage resistance which are permanent to washing with soap and alkali.

#### Example 8

100 parts of methylol cyclo propylstearamide are added gradually to a mixture of 45 parts of carbon tetrachloride and 91 parts of phosphorus trichloride. One hour after all the methylol amide has been added 40 parts of acetic acid are added and the reaction mixture is allowed to stand at room temperature for four days. The reaction mixture gradually becomes viscous and at the same time soluble in dilute alkali. The reaction mixture, which now contains the phosphonichloride, is treated with aqueous hydrogen chloride of 8 percent strength at about 50° C.

70

and yields a crystalline, readily filterable product which may be recrystallized from alcohol, and which is readily soluble in dilute alkali and in hot water. This product is cyclo propylstear amidomethyl phosphonic acid,



10 Cotton fabric is treated with an aqueous 4 percent solution of the ammonium salt of the above phosphonic acid and then heated at not over 150° C. for a few minutes. The fabric acquires a soft feel and is strongly water repellent. These properties are not lost when the fabric is washed. The fabric is also crease-resistant.

#### Example 9

One mole of cyclopropionyl urea (which may be prepared by condensing cyclopropionic acid with urea) is suspended in 125 parts of ethylene dichloride with one mole paraformaldehyde, one mole of dimethyl ethyl amine hydrochloride and 0.4 part triethyl amine. The mixture is warmed 25 for five hours at 60° C., with stirring. Upon removal of the solvents a water soluble product is obtained which dissolves in warm water to form a somewhat cloudy solution having foaming properties. This product is believed to have the 30 formula:



35 When the aqueous solution of this product is made alkaline, a precipitate is quickly formed which is insoluble in methanol or acidified water.

Cotton or wool material is impregnated with an aqueous solution of this product, dried at about 60 to 80° C. and then heated to a temperature between 100 and 150° C. in an oven with rapid circulation. The material acquires a water repellent finish which is permanent in the sense that it is not removed by laundering with 45 soap and alkali.

#### Example 10

50 A mixture of pyridine hydrochloride and pyridine is made by passing gaseous hydrogen chloride into 100 parts of pyridine until an increase in weight of 9.1 parts is obtained. To this mixture are added one mole of paraformaldehyde and one mole of



55 The mixture is stirred and heated at 60° C. for 4 hours. The reaction mass is then cooled and 60 mixed with an equivalent amount of ethyl ether, and the lower oily layer which separates is removed and washed with a further quantity of ether. The washed oil is then shaken up with cold chloroform, allowed to stand and the lower layer separated off and washed with ether. The 65 quaternary pyridinium salt is obtained, corresponding to the formula:



This compound is dissolved in water to give a 4 percent solution, which is then applied to a spun rayon challis to a 100 percent pick-up by weight. The fabric is dried at 90° C. and then baked at 120° C. for ten minutes. The resulting product has permanent water repellency and dimensional stability, and is crease-resistant.

*Example 11*

One mole of cyclopropyl octamethylene alcohol and one mole of paraformaldehyde are suspended in 120 parts of dry benzene. Gaseous hydrogen chloride is passed into the stirred mixture, keeping the temperature below 10° C. until a clear benzene solution is obtained. The lower aqueous layer is then removed and the upper benzene layer dried with calcium chloride. The benzene is removed and the residue recovered. The new compound is believed to have the formula:



This product is dissolved in dry pyridine. The solid pyridinium chloride is readily soluble in water and alcohol.

Sufficient compound is dissolved in water to give a 3 percent solution, which is then applied to 100 percent wool and cotton fabrics at room temperature. The fabrics are dried at 50° C. and then baked at not over 150° C. for 20 minutes. The products are permanently water repellent and dimensionally stable.

*Example 12*

One mole of cyclopropionamide is heated with 0.6 mole of chloromethyl ethyl ether for 3½ hours at 90° C. with stirring, at which time evolution of hydrogen chloride is complete. Excess chloromethyl ether is removed by distillation. The residue is dissolved with one mole of paraformaldehyde in benzene and heated until when a test portion is cooled, no solid is seen to separate. The mixture is allowed to settle and the benzene solution is removed from the lower aqueous layer. The benzene is then distilled off under reduced pressure and the dichloromethyl compound recovered. This is dissolved in 200 parts of ethyl acetate and the solution mixed with an excess of pyridine. A white precipitate is obtained which is filtered off and dried. The white powder thus recovered dissolves in hot water, forming a clear, foaming solution, and is soluble in alcohol and in hot benzene and acetone. The compound appears to have the formula:



This compound is dissolved in water to give a 4 percent solution, which is then applied to rayon and cotton fabrics at room temperature to a 100 percent pickup. The fabrics are dried at 75° C. and then baked at 125° C. for 15 minutes. The products possess a permanent water repellency and dimensional stability, and are crease-resistant.

*Example 13*

A solution is made by dissolving 100 parts of urea in 200 parts of neutralised aqueous form-

aldehyde solution (40 percent), to which is added 7.5 parts of concentrated ammonia solution (Sp. Gr. 0.880). The mixture is boiled for a few minutes and then rapidly cooled to room temperature. There are now added 6 parts of ammonium dihydrogen phosphate and 8 parts of cyclopropionyl ureido methylene pyridinium chloride in the form of an aqueous suspension in 50 parts of cold water and the mixture is diluted to a total volume of 400 parts by addition of cold water.

Cotton sheeting is padded in the above solution at room temperature and is then squeezed so that it contains its own weight of impregnating solution. It is then dried in a current of warm air at 40°-50° C. The dry fabric is heated for a few minutes at not over 150° C. Finally it is washed for a few minutes at 45° C. in a solution containing 2 parts of soap and 1 part of anhydrous sodium carbonate in 1000 parts of water, well rinsed in warm water and dried.

The fabric now has a remarkably soft handle, is highly water repellent and is crease-resistant. These properties survive washing and dry cleaning treatments.

*Example 14*

A sufficient quantity of cyclopropyl octa methylene pyridinium chloride is dissolved in water to give an 8 percent solution. A rayon fabric is padded with the solution to a 100 percent pick-up by weight, dried at 60° C. and then baked at 120° C. for 10 minutes. The resulting product is dimensionally stable, showing no shrinkage even after repeated washings, and is permanently water repellent.

*Example 15*

Ten parts by weight of cyclopropyl carboxyethylene oxymethylene pyridinium chloride



(prepared from cyclopropyl methyl ketone, paraformaldehyde and pyridine in the presence of dry HCl) are dissolved in 30 parts of hot 95 percent ethyl alcohol and diluted with 100 parts of warm water. 80 x 80 cotton cloth and spun rayon challis cloth are padded in the solution passed between rollers set to retain a weight of solution equal to the weight of the cloth, dried at 80° C. and cured by heating in an oven for about 15 minutes at not over 150° C., washed 15 minutes in a one percent soap solution and then dried. Both samples of treated cloth are then very soft and have excellent water repellency and dimensional stability.

The following is claimed:

1. Compounds having the general formula:



where R is a bivalent radical selected from the group consisting of

$\begin{array}{c} \text{NH} \\ | \\ -\text{O}-, -\text{CO}-, -\text{COO}-, -\text{CONH}-, -\text{CO}-, -\text{NHCOO}-, \\ -\text{NHCNH}-, -\text{CONHCONH}-, -\text{OCH}_2\text{NHCONH}- \\ \text{and} -\text{CH}_2\text{OOCNH}-, \text{A is a hydrocarbon radical} \\ \text{containing from 1 to 20 carbon atoms, N(tert) is} \\ \text{pyridine, X is an anion and } m, n, \text{ and } p \text{ are numbers} \\ \text{selected from the numbers 0 and 1, provided that } m, n \text{ and } p \text{ cannot all be 0 and that} \\ \text{when } m \text{ and } n \text{ are both 1, } p \text{ is also 1.} \end{array}$

## 15

2. Quaternary ammonium compounds having the formula



wherein  $n$  is an integer from 1 to 20, and  $\text{X}$  is an anion.

3. Quaternary ammonium compounds having the formula:



wherein  $n$  is an integer from 1 to 20 and  $\text{X}$  is an anion.

4.



wherein  $n$  is an integer from 1 to 20 and  $\text{X}$  is an anion.

5. A process for treating organic textile materials to enhance the water repellency, crease-proofness and dimensional stability thereof which comprises impregnating said material with a solution of a compound having the general formula:



where  $\text{R}$  is a radical selected from the group consisting of

35



## 16

and  $-\text{CH}_2\text{OOCNH}-$ ,  $\text{A}$  is a hydrocarbon radical containing from 1 to 20 carbon atoms,  $\text{N}(\text{tert})$  is the residue of a tertiary amine,  $\text{X}$  is an anion and  $m$ ,  $n$ , and  $p$  are numbers selected from the numbers 0 and 1, provided that  $m$ ,  $n$  and  $p$  cannot all be 0 and that when  $m$  and  $n$  are both 1,  $p$  is also 1, said solution being applied in sufficient amounts to cause from 0.05 to 20 per cent of said compound to be deposited on said material based on the weight of the material when dry, said solution having a pH of from 5 to 10 and a temperature of below 40° C., drying said impregnated material at a temperature of from 30 to 80° C. and heating the material to a temperature from 80° to 200° C.

6. The process as in claim 5 wherein said organic textile material is cellulosic.

7. The textile material made by the process of claim 5.

20

## References Cited in the file of this patent

## UNITED STATES PATENTS

| Number    | Name               | Date           |
|-----------|--------------------|----------------|
| 2,125,901 | Evans et al. ----- | Aug. 9, 1938   |
| 2,131,362 | Baldwin -----      | Sept. 27, 1938 |
| 2,148,392 | Baldwin -----      | Feb. 7, 1939   |
| 2,189,664 | Katzman -----      | Feb. 6, 1940   |
| 2,209,383 | Bock -----         | July 30, 1940  |
| 2,291,021 | Bock -----         | July 28, 1942  |

## FOREIGN PATENTS

| Number  | Country             | Date           |
|---------|---------------------|----------------|
| 547,846 | Great Britain ----- | Sept. 15, 1942 |

30

35